

# United States Patent Office

3,420,732

Patented Jan. 7, 1969

1

3,420,732

TRANSFER FILM AND PROCESS OF USING SAME  
Larry J. Bresina, St. Paul, and Richard A. Miller, White  
Bear Lake, Minn., assignors to Minnesota Mining and  
Manufacturing Company, St. Paul, Minn., a corpora-  
tion of Delaware  
No Drawing, Filed Oct. 23, 1965, Ser. No. 504,055  
U.S. Cl. 161—227 13 Claims  
Int. Cl. G03c 11/00

This invention relates to an electrophotographic copy-  
sheet which can be retouched with water soluble dyestuffs.  
In one aspect this invention relates to color retouchable  
electrolytic electrophotographic full color prints. In an-  
other aspect this invention relates to a transfer film for  
providing a retouchable surface on an electrophotographic  
print.

One electrophotographic method for providing full  
color reproductions of a light image utilizes electrolytic  
electrophotographic techniques. As described in U.S.  
3,010,884 and 3,130,655 successive deposits of subtractive  
primary colors may be applied to the light exposed  
surface of an electrolytically developable photoconductive  
copsheet. Particularly suitable color developers include  
basic nitrogen containing organic compounds which are  
soluble in an aqueous acidic solution and which are in-  
soluble in water at a pH above 7, as shown in U.S.  
3,172,827. Another class of outstanding color developers  
are the water soluble onium cations which decompose  
electrolytically to form water insoluble compounds, as  
shown in U.S. 3,172,826. Although frequently it is desir-  
able to retouch finished full color prints, as in conven-  
tional color photography, the print surfaces of most  
electrolytic electrophotographic copsheets are not gen-  
erally sufficiently receptive to the water soluble dyestuffs  
preferred for color retouching. Although it is possible to  
provide a gelatin retouchable layer over the final color  
print, gelatin is susceptible to water spotting, becomes  
tacky when wet, embrittles at lower temperatures, is sensi-  
tive to actinic radiation, and tends to curl with changes  
in humidity.

It is an object of this invention to provide an electro-  
photographic copsheet with a surface which can be color  
retouched with aqueous solutions of water soluble dye-  
stuffs.

Another object of this invention is to provide a trans-  
fer film suitable for application to the surface of an  
electrophotographic print to provide a retouchable sur-  
face.

A further object of this invention is to provide a method  
for rendering an electrophotographic print retouchable  
with water soluble dyestuffs.

Other objects and advantages will be apparent from  
the following description.

In accordance with this invention it has been found  
that an electrophotographic copsheet having a visible  
image thereon can be rendered readily retouchable with  
water soluble dyestuffs without loss of other desirable  
physical properties if a layer of an essentially colorless  
methanol soluble synthetic polyamide is bonded to the  
image bearing copsheet surface. A preferred class of  
methanol soluble polyamides is the nitrogen substituted  
polyamides, particularly the N-alkoxymethyl polyamides,  
as described in U.S. 2,412,993, 2,430,860, 2,430,907 and  
2,441,057. Other suitable methanol soluble synthetic poly-  
amides include polyamides prepared with the use of cer-  
tain diamines, e.g. triglycoldiamine, and multicomponent  
systems, e.g. interpolyamides of hexamethylene diammonium  
adipate, hexamethylene diammonium sebacate and  
caprolactam ("Zytel 61," a product of E. I. du Pont de  
Nemours and Co.). By "methanol soluble polyamide" is  
meant a polyamide which can exist as at least a 5 percent

2

solution or gel in methanol at 25° C. The methanol sol-  
uble polyamides provide a retouchable surface for elec-  
trophotographic prints without the problems of curl and  
tackiness encountered in conventional prints. In the form  
of a retouchable layer having a thickness below about 5  
mils they improve color saturation and appearance of the  
image and serve also to protect the print from abrasion,  
water spotting and degradation by actinic light.

The retouchable layer may be prepared by coating the  
electrophotographic print with a methanol-water solution  
of the methanol soluble polyamide. However, it is more  
convenient to provide a transfer film which comprises a  
transparent layer of methanol soluble polyamide on a  
releasable or strippable backing. Various backing mate-  
rials with dry releasability from the polyamide may be  
used, such as a polypropylene film with or without a  
silica slip agent, polyethylene terephthalate, polypropylene  
coated paper, polyethylene coated paper, polyethylene  
film and poly-methyl methacrylate coated paper. To im-  
prove the adhesion of the methanol soluble polyamide  
retouchable layer to the print surface a suitable essen-  
tially colorless adhesive system, e.g. solvent and/or heat  
activatable adhesives and pressure sensitive adhesives,  
can be employed. If a heat activatable adhesive is used,  
it should generally be capable of activation at a tem-  
perature below about 120° C., preferably below 95° C.,  
to avoid degradation of the print. The adhesive may be  
coated directly onto the print surface before application  
of the retouchable film or it may be carried on the sur-  
face of the retouchable film and form an integral com-  
ponent of the transfer film construction. Because of its  
relative ease in application the adhesive containing trans-  
fer film is preferred, generally with a releasable outer  
layer or liner to protect the adhesive prior to use if a  
pressure sensitive formulation is utilized. The surface of  
the retouchable film can be varied in texture from glossy  
to matte by selecting a release backing with the desired  
finish or by incorporating colloidal silica into the retouch-  
able layer. Frequently it is desirable to include a sur-  
factant into the retouchable layer or into the solution of  
retouching dyestuff to improve the rate and uniformity  
of dye absorption.

The following examples will illustrate the invention.

## Example 1

A methanol soluble polyamide (B.C.I. nylon 819,  
N-methoxymethyl polyhexamethylene adipamide, 500-  
600% ultimate elongation, 3400-3600 p.s.i. tensile  
strength, 12.4% water absorption, melting range 140-  
148° C., tack point 130° C.) was coated from the fol-  
lowing solution onto a 5 mil polypropylene film to  
provide a dry film of one mil thickness.

|                          | Grams |
|--------------------------|-------|
| Trichloroethylene        | 23.3  |
| Methanol                 | 56.2  |
| Polyamide                | 18.7  |
| Water solution (30%) of: |       |

60  1.2

(60% by weight of combined ethylene oxide)

65 Onto the dry polyamide surface a 24% solution of  
polyvinyl acetate (9% hydrolyzed) in toluene was coated  
to serve as a heat activatable adhesive, the dry coating  
thickness being one mil. The resulting transfer film was  
laminated by means of heated squeeze rolls at a tem-  
perature of about 80° C. to an electrophotographic full  
color print. After lamination the polypropylene release  
film was dry stripped from the print, exposing a semi-  
gloss polyamide surface. A 5 weight percent aqueous

solution of Genacryl Red 6B (Color Index No. 48020) containing 0.25 weight percent of



was applied to the white areas of the topcoated print for 15 seconds. After removal of excess dye the dyed areas had a green reflection optical density of 2.40 (Wratten filter No. 93).

Example 2

A polymethyl methacrylate coated paper was coated with the following solution to give a dry film thickness of one mil.

|                                                                                                                                                                                              | Grams |
|----------------------------------------------------------------------------------------------------------------------------------------------------------------------------------------------|-------|
| Methylene chloride -----                                                                                                                                                                     | 25    |
| Methanol -----                                                                                                                                                                               | 60    |
| N - methoxymethyl polyhexamethylene adipamide (500-600% ultimate elongation, 3800-4000 p.s.i. tensile strength, 10.0% water absorption, melting range 145-153° C., tack point 135° C.) ----- | 20    |

A colorless polyester high strength adhesive (Du Pont 46950 polyester adhesive) was coated onto the polyamide surface (dry coating thickness of one mil). The resulting construction was laminated by means of heated squeeze rolls at a temperature of about 80° C. to an electrophotographic print. After lamination the methylmethacrylate coated paper was stripped from the print leaving a surface with a pleasing semigloss texture. A 5 weight percent aqueous solution of Pontamine Sky Blue 6BX (Color Index No. 24410) containing 0.25%



was applied to a white area of the print surface for 15 seconds. In the dyed area both the red and green reflection optical density was 1.74 (Wratten filter Nos. 92 and 93, respectively) after the excess dye was removed.

Example 3

A retouchable layer was prepared by coating an electrophotographic print with the following solution:

|                              | Grams |
|------------------------------|-------|
| Methanol -----               | 65    |
| Water -----                  | 15    |
| Polyamide of Example 1 ----- | 20    |

The dry thickness of the retouchable layer was 0.5 mil. A 5 weight percent aqueous solution of Calcocid Blue AX Double (Color Index No. 42080) was applied to a white area of the print for 15 seconds. The excess dye was washed off, and the dyed area had a reflection optical density of 1.33 measured through a Kodak Wratten filter No. 92.

Various other embodiments of the present invention will be apparent to those skilled in the art without departing from the scope thereof.

We claim:

1. A dimensionally stable, electrophotographic print having bonded to its image bearing surface an essentially colorless, methanol soluble, synthetic polyamide layer.

2. The electrophotographic print of claim 1 in which

said essentially colorless, methanol soluble, synthetic polyamide layer is adhesively bonded to said print surface.

3. The electrophotographic print of claim 1 in which said essentially colorless, methanol soluble, synthetic polyamide layer is bonded to said print surface with a heat activated, essentially colorless adhesive.

4. In an electrophotographic print the improvement which comprises an essentially colorless, methanol soluble, synthetic polyamide layer bonded to the surface of said print, said layer being retouchable with water soluble dyestuffs.

5. The electrophotographic print of claim 4 in which said methanol soluble, synthetic polyamide is an N-alkoxymethyl polyamide.

6. A transfer film for rendering an electrophotographic print retouchable with water soluble dyestuffs which comprises an essentially colorless, methanol soluble, synthetic polyamide film releasably bonded to a support sheet.

7. The transfer film of claim 6 in which said polyamide film contains a heat activatable adhesive on its exposed surface.

8. The transfer film of claim 6 in which said polyamide film contains on its exposed surface an adhesive capable of heat activation at a temperature below about 120° C.

9. The transfer film of claim 6 in which said polyamide film contains on the surface opposite said releasable support sheet an adhesive layer over which is superimposed a protective liner which can be stripped from said adhesive layer without removal of adhesive from the polyamide layer.

10. The transfer film of claim 6 in which said polyamide film contains on its exposed surface a solvent activatable adhesive.

11. The process for rendering an electrophotographic print retouchable with water soluble dyestuffs which comprises providing an essentially colorless, methanol soluble, synthetic polyamide layer on the print surface.

12. The process for rendering an electrophotographic print retouchable with water soluble dyestuffs which comprises coating the print surface with a solution of an essentially colorless, methanol soluble, synthetic polyamide and drying the resulting coating.

13. The process for rendering an electrophotographic print retouchable with water soluble dyestuffs which comprises (1) contacting the print surface with a transfer film comprising a layer of an essentially colorless, methanol soluble, synthetic polyamide releasably bonded to a support sheet, said support sheet being furthermore from said print surface, (2) bonding said polyamide layer to said print surface, and (3) removing said support sheet from said polyamide layer without breaking the bond between said print surface and said polyamide layer.

References Cited

UNITED STATES PATENTS

3,143,416 8/1964 Reichel et al. ----- 96-35

EARL M. BERGERT, Primary Examiner.

60 M. L. KATZ, Assistant Examiner.

U.S. Cl. X.R.

156-239;117-3.4, 161; 260-78